# EUROPEAN PATENT SPECIFICATION

(11) **EP 1 409 613 B1**
(45) Date of publication and mention of the grant of the patent: **13.09.2006**
(21) Application number: 02748783.4
(22) Date of filing: 13.06.2002
(51) Int. Cl.: C10G 73/44

(54) **PROCESS FOR PREPARING A MICROCRYSTALLINE WAX**
VERFAHREN ZUR HERSTELLUNG EINES MIKROKRISTALLINEN WACHSES
METHODE DE PREPARATION D'UNE CIRE MICROCRISTALLINE

(30) Priority: 15.06.2001 EP 01202313
(43) Date of publication of application: 21.04.2004
(62) Divisional of application: 04102821.8
(73) Proprietor: SHELL INTERNATIONALE RESEARCH MAATSCHAPPIJ B.V., 2596 HR Den Haag (NL)
(72) Inventor: HOEK, Arend, NL-1031 CM Amsterdam (NL); SCHADENBERG, Hendrik, NL-1031 CM Amsterdam (NL)
(86) International application number: PCT/EP2002/006584
(87) International publication number: WO 2002/102941

(56) References cited:
- WO-A1-01/74969
- DE-A- 2 644 519
- GB-A- 1 245 187
- US-A- 2 668 866
- US-A- 4 139 494
- US-A- 4 186 078
- US-A- 4 239 546
- US-A- 4 415 649
- US-A- 4 839 422

## Description

The invention is related to a process for preparing a microcrystalline wax.

It is known to prepare a microcrystalline wax product by means of solvent dewaxing of a petroleum fraction boiling in the base oil range. Examples of such processes are described in The Petroleum Handbook, 6th edition, Elsevier, 1983, Chapter 5 page 265.

It is also known to prepare wax from the product obtained from the Fischer-Tropsch process as for example described in Naidoo P., Watson M.D., Manufacturing and quality aspects of producing hard waxes from natural gas and the resulting HMA performance obtained when using such a wax, 1994 Hot Melt Symposium, TAPPI Proceedings, pages 165-170.

A disadvantage of such a wax based on a Fischer-Tropsch product is that it is too hard to be used in applications as for example in specific hot melt adhesives, as lubricant in PVC manufacturing, chewing gum, petroleum gel, pharmaceutical products, cosmetics, textile impregnation and paper coating applications. The hardness of a wax may be measured by the IP 376 method. Typical PEN values at 43 °C as obtained using this method on commercially available Fischer-Tropsch derived waxes are between 0.2 and 0.6 mm.

WO-A-0174969 discloses a process to prepare Fischer-Tropsch derived waxes having a high needle penetration value by hydroisomerisation of the entire wax product obtained in the Fischer-Tropsch synthesis.

It is an object of the present invention to provide a process to prepare a microcrystalline wax having the desired properties, especially having a PEN value (IP 376) at 43 °C of above 0.8 mm.

This object is achieved by the following process. Process to prepare a microcrystalline wax by contacting under hydroisomerisation conditions a feed, comprising at least 80 wt% of normal-paraffins, having a congealing point of between 95 and 125 °C and a PEN at 43 °C as determined by IP 376 smaller than 0.7 mm, with a catalyst comprising a noble metal and a porous silica-alumina carrier.

Preferably the hydroisomerisation conditions are so chosen that preferably less than 10 wt%, and more preferably less than 5 wt%, of the compounds in the feed boiling above 370 °C are converted to products boiling below 370 °C. The temperature is suitably between 200 and 400 °C and preferably between 250 and 350 °C. The hydrogen partial pressure is suitably between 10 and 100 bar and preferably between 30 and 60 bar. The weight hourly space velocity is suitably between 0.5 and 5 kg/l/h.

The noble metal as present in the catalyst is preferably platinum, palladium or a combination of said metals. The content of noble metal in the catalyst is suitably between 0.1 and 2 wt% and preferably between 0.2 and 1 wt%.

The catalyst carrier may comprise any suitable amorphous silica-alumina. The amorphous silica-alumina preferably contains alumina in an amount in the range of from 2 to 75% by weight, more preferably from 10 to 60% by weight. A very suitable amorphous silica-alumina product for use in preparing the catalyst carrier comprises 45% by weight silica and 55% by weight alumina and is commercially available (ex. Criterion Catalyst Company, USA).

More preferably the amorphous silica-alumina carrier has a certain degree of macroporous pores. The macroporosity of the carrier is suitably in the range of from 5% vol to 50% vol, wherein the macroporosity is defined as the volume percentage of the pores having a diameter greater than 100 nm. More preferably the carrier has a macroporosity of at least 10% vol, even more preferably at least 15% vol and most preferably at least 20% vol. Especially preferred catalysts for use in the process comprise a carrier having a macroporosity of at least 25% vol. Catalysts comprising carriers having a high macroporosity may suffer the disadvantage that the catalyst has a low resistance to damage by crushing. Accordingly, the macroporosity is preferably no greater than 40% vol, more preferably no greater than 38% vol, even more preferably no greater than 35% vol. The side crushing strength of the catalyst is suitably above 75 N/cm, more preferably above 100 N/cm. The bulk crushing strength of the catalyst is suitably above 0.7 MPa, more preferably above 1 MPa.

References to the total pore volume are to the pore volume determined using the Standard Test Method for Determining Pore Volume Distribution of Catalysts by Mercury Intrusion Porosimetry, ASTM D 4284-88, at a maximum pressure of 4000 bar, assuming a surface tension for mercury of 484 dyne/cm and a contact angle with amorphous silica-alumina of 140°. The total pore volume of the carrier as measured by the above method, is typically in the range of from 0.6 to 1.2 ml/g, preferably in the range of from 0.7 to 1.0 ml/g, more preferably in the range of from 0.8 to 0.95 ml/g.

It will be appreciated that a major portion of the total pore volume is occupied by pores having a pore diameter smaller than 100 nm, that is meso- and micropores. Typically, a major portion of those meso- and micropores has a pore diameter in the range of from 3.75 to 10 nm. Preferably, from 45 to 65% vol of the total pore volume is occupied by pores having a pore diameter in the range of from 3.75 to 10 nm.

In addition to amorphous silica-alumina, the carrier may also comprise one or more binder materials. Suitable binder materials include inorganic oxides. Both amorphous and crystalline binders may be applied. Examples of binder materials comprise silica, alumina, clays, magnesia, titania, zirconia and mixtures thereof. Silica and alumina are preferred binders, with alumina being especially preferred. The binder, if incorporated in the catalyst, is preferably present in an amount of from 5 to 50% by weight, more preferably from 15 to 40% by weight, on the basis of total weight of the carrier Catalysts comprising a carrier without a binder are preferred for use in the process of this invention. The above preferred catalyst can be obtained by the process as for example described in EP-A-666894. Further examples of suitable catalysts are described in WO-A-200014179, EP-A-532118, EP-A-587246, EP-A-532116, EP-A-537815 and EP-A-776959.

The feed comprises at least 80 wt%, and preferably at least 85 wt%, of normal-paraffins. The feed has a congealing point of above 95 °C. The upper limit for the melting temperature and congealing point is below 125 °C. The PEN value as determined by IP 376 at 43 °C is preferably smaller than 0.7 mm. The oil content as determined by ASTM D 721 will typically be low, for example smaller than 1 wt% and more typically less than 0.5 wt%. The kinematic viscosity at 150 °C of the feed is preferably above 7 cSt. The feed suitably contains less than 0.1 ppm sulphur in order not to deactivate the catalyst.

Such a preferred feed is suitably obtained in a Fischer-Tropsch synthesis. Such a process can prepare fractions having a high content of normal paraffins. Examples of such processes are the so-called commercial Sasol process, the commercial Shell Middle Distillate Process or by the non-commercial Exxon process. These and other processes are for example described in more detail in EP-A-776959, EP-A-668342, US-A-4943672, US-A-5059299, WO-A-9920720. A preferred Fischer-Tropsch process to prepare the feed for the present process is described in WO-A-9934917. This process is preferred because it yields a Fischer-Tropsch product, comprising a sufficient amount of the fraction having a congealing point of between 95 and 125°C.

Examples of commercially available Fischer-Tropsch derived wax products which can be used as feedstock are SX100 as described in "The Markets for Shell Middle Distillate Synthesis Products", Presentation of Peter J.A. Tijm, Shell International Gas Ltd., Alternative Energy '95, Vancouver, Canada, May 2-4, 1995 and Paraflint H1 as marketed by Schümann Sasol Ltd (SA).

The synthesis product as directly obtained in the Fischer-Tropsch process is preferably hydrogenated in order to remove any oxygenates and saturate any olefinic compounds present in such a product. Such a hydrotreatment is described in for example EP-B-668342. The feed for the present product can be obtained by separating the lower boiling compounds and optionally higher boiling compounds from the Fischer-Tropsch product by means of distillation or any other suitably separation technique.

The microcrystalline wax as obtained by the present process, optionally after a de-oiling step, may find application in the earlier mentioned applications. The wax may be used as a lubricant for processing of PVC (poly vinyl chloride), for example for rigid PVC extrusion. The wax may also be used as a carrier wax for polytheylene master batches. Furthermore it has been found that the wax product has a better compatible with polar compounds as compared to the feed. For example the wax product is better compatible with polar pigments.

The invention is also directed to the soft microcrystalline wax as such having the following properties. Fischer-Tropsch derived wax having a congealing point as determined by ASTM D 938 of between 85 and 120 and more preferably between 95 and 120 °C and a PEN at 43 °C as determined by IP 376 of more than 0.8 mm and preferably more than 1 mm. The wax is further characterized in that it preferably comprises less than 1 wt% aromatic compounds and less than 10 wt% naphthenic compounds, more preferably less than 5 wt% naphthenic compounds. The mol percentage of branched paraffins in the wax is preferably above 33 and more preferably above 45 and below 80 mol% as determined by C₁₃ NMR. This method determines an average molecular weight for the wax and subsequently determines the mol percentage of molecules having a methyl branch, the mol percentage of molecules having an ethyl branch, the mol percentage of molecules having a C₃ branch and the mol percentage having a C₄⁺ branch, under the assumption that each molecule does not have more than one branch. The mol% of branched paraffins is the total of these individual percentages. This method calculated the mol% in the wax of an average molecule having only one branch. In reality paraffin molecules having more than one branch may be present. Thus the content of branched paraffins determined by different method may result in a different value.

The oil content as determined by ASTM D 721 is typically below 2 wt%. The lower limit is not critical. Values of above 0.5 wt% may be expected, but lower values can be achieved depending on the method in which the wax is obtained. Most likely the oil content will be between 1 and 2 wt%. The kinematic viscosity at 150 °C of the wax is preferably higher than 8 cSt and more preferably higher than 12 and lower than 18 cSt.

The invention will now be illustrated with the following non-limiting examples.

### Example 1

A wax fraction as obtained from the Fischer-Tropsch synthesis product as obtained in Example VII using the catalyst of Example III of WO-A-9934917 was continuously fed to a hydroisomerisation step. The properties of the feed are described in Table 1.

In the hydroisomerisation step the fraction was contacted with a hydroisomerisation catalyst of Example 1 of EP-A-532118. The hydroisomerisation step was performed at 30 bara and at a temperature of 325 °C. The remaining conditions were so chosen that the conversion of the feed to products boiling below 370 °C was below 10 wt%.

The product as obtained in the hydroisomerisation were analysed and the results are presented in Table 1.

**Table 1**

| | SX100* | Paraflint H1** | feed | Product |
|---|---|---|---|---|
| Congealing point (ASTM D 938; °C) | 97.3 | 100 | 104.5 | 101.0 |
| Drop melting point (ASTM D 127) (°C) | 110.0 | 113.5 | 116.7 | 113.4 |
| PEN at 25 °C (IP 376) (mm) | 0.1 | 0.1 | 0.1 | 0.8 |
| PEN at 43 °C | 0.4 | 0.4 | 0.2 | 1.6 |
| PEN at 65 °C | 1.1 | 1.7 | 0.7 | 4.0 |
| Oil content (ASTM D 721; wt%) | < 0.1 | Not measured | < 0.1 | 1.6 |
| Kinematic viscosity at 150 °C (ASTM D 445) | 7.97 | Not measured | 14 | 13.8 |
| Crystal structure by microscopic observation | Yes | Yes | Yes | Yes |
| % branching (mol%) | 9 | 11.5 | 11.1 | 60*** |

| | | | | |
|---|---|---|---|---|
| * SX100 is a Fischer-Tropsch wax as marketed by Shell Malaysia bhp | | | | |
| ** Paraflint H1 is a Fischer-Tropsch derived wax marketed by Schumann Sasol | | | | |
| *** 36 mol% mono-methyl branched paraffin molecules, 8 mol% mono-ethyl branched paraffin molecules, 4 mol% mono-propyl branched paraffin molecules and 12 C₄⁺ mono-branched paraffin molecules. | | | | |

## Claims

1. Process to prepare a microcrystalline wax by contacting under hydroisomerisation conditions a feed, comprising at least 80 wt% of normal-paraffins, having a congealing point of between 95 and 125 °C and a PEN at 43 °C as determined by IP 376 smaller than 0.7 mm, with a catalyst comprising a noble metal and a porous silica-alumina carrier.

2. Process according to claim 1, wherein less than 10 wt% of the compounds in the feed boiling above 370 °C are converted to products boiling below 370 °C.

3. Process according to claim 2, wherein less than 5 wt% of the compounds in the feed boiling above 370 °C are converted to products boiling below 370 °C.

4. Process according to any one of claims 1-3, wherein the hydroisomerisation conditions comprise a temperature of between 250 and 350 °C, a hydrogen partial pressure of between 30 and 60 bar and a weight hourly space velocity of between 0.5 and 5 kg/l/h.

5. Process according to any one of claims 1-4, wherein the noble metal is platinum, palladium or a combination of said metals.

6. Process according to any one of claims 1-5, wherein the amorphous silica-alumina carrier has a macroporosity in the range of from 5% vol to 50% vol, wherein the macroporosity is defined as the volume percentage of the pores having a diameter greater than 100 nm.

7. Process according to claim 6, wherein the macroporosity is between 10 and 40% vol.

8. Process according to any one of claims 1-7, wherein the amorphous silica-alumina carrier comprises alumina in an amount in the range of from 2 to 75% by weight.

9. Process according to claim 8, wherein the alumina content is between 10 to 60% by weight.

10. Process according to any one of claims 1-9, wherein the total pore volume of the carrier is in the range of from 0.6 to 1.2 ml/g.

11. Process according to any one of claims 1-10, wherein the feed is obtained by means of a Fischer-Tropsch synthesis.

12. Use of a wax as obtained in a process according to any one of claims 1-11 as a solidifier component in a hot melt adhesive.

13. Use of a wax as obtained in a process according to any one of claims 1-11 as a lubricant in PVC processing.

14. Use of a wax as obtained in a process according to any one of claims 1-11 as a gloss aid in a cosmetic composition.

## Patentansprüche

1. Verfahren zur Herstellung eines mikrokristallinen Wachses durch Inkontaktbringen eines Einsatzmaterials unter Hydroisomerisierungsbedingungen, welches Einsatzmaterial wenigstens 80 Gew.-% an Normalparaffinen umfaßt, mit einem Erstarrungspunkt von 95 bis 125°C und einem PEN-Wert bei 43°C, bestimmt mittels IP 376, von weniger als 0,7 mm, mit einem ein Edelmetall und einen porösen Siliciumoxid-Aluminiumoxid-Träger umfassenden Katalysator.

2. Verfahren nach Anspruch 1, worin weniger als 10 Gew.-% der Verbindungen im Einsatzmaterial, welche über 370°C sieden, in Produkte, welche unter 370°C sieden, umgewandelt werden.

3. Verfahren nach Anspruch 2, worin weniger als 5 Gew.-% der Verbindungen im Einsatzmaterial, welche über 370°C sieden, in Produkte, welche unter 370°C sieden, umgewandelt werden.

4. Verfahren nach einem der Ansprüche 1 bis 3, worin die Hydroisomerisierungsbedingungen eine Temperatur von 250 bis 350°C, einen Wasserstoffpartialdruck von 30 bis 60 bar und eine gewichtsbezogene stündliche Raumgeschwindigkeit von 0,5 bis 5 kg/l/h umfassen.

5. Verfahren nach einem der Ansprüche 1 bis 4, worin das Edelmetall Platin, Palladium oder eine Kombination dieser Metalle ist.

6. Verfahren nach einem der Ansprüche 1 bis 5, worin der amorphe Siliciumoxid-Aluminiumoxid-Träger eine Makroporosität im Bereich von 5 Vol.-% bis 50 Vol.-% aufweist, wobei die Makroporosität als der Volumsprozentsatz der Poren mit einem Durchmesser von mehr als 100 nm definiert ist.

7. Verfahren nach Anspruch 6, worin die Makroporosität von 10 Vol.-% bis 40 Vol.-% beträgt.

8. Verfahren nach einem der Ansprüche 1 bis 7, worin der amorphe Siliciumoxid-Aluminiumoxid-Träger Aluminiumoxid in einer Menge im Bereich von 2 bis 75 Gew.-% umfaßt.

9. Verfahren nach Anspruch 8, worin der Aluminiumoxidgehalt von 10 bis 60 Gew.-% beträgt.

10. Verfahren nach einem der Ansprüche 1 bis 9, worin das Gesamtporenvolumen des Trägers im Bereich von 0,6 bis 1,2 ml/g beträgt.

11. Verfahren nach einem der Ansprüche 1 bis 10, worin das Einsatzmaterial mittels einer Fischer-Tropsch-Synthese erhalten wird.

12. Verwendung eines Wachses, wie es in einem Verfahren nach einem der Ansprüche 1 bis 11 erhalten wird, als Verfestigungskomponente in einem Heißschmelzkleber.

13. Verwendung eines Wachses, wie es in einem Verfahren nach einem der Ansprüche 1 bis 11 erhalten wird, als Schmiermittel in der PVC-Verarbeitung.

14. Verwendung eines Wachses, wie es in einem Verfahren nach einem der Ansprüche 1 bis 11 erhalten wird, als Glanzhilfsmittel in einer kosmetischen Zusammensetzung.

## Revendications

1. Procédé de préparation d'une cire microcristalline par mise en contact, dans des conditions d'hydroisomérisation, d'une charge d'alimentation comprenant au moins 80% en poids de paraffines normales ayant un point de congélation compris entre 95 et 125°C et une valeur PEN à 43°C, déterminée selon IP 376, de moins de 0,7 mm, avec un catalyseur comprenant un métal noble et un support poreux de silice - alumine.

2. Procédé selon la revendication 1, dans lequel moins de 10% en poids des composés de la charge ayant un point d'ébullition de plus de 370°C sont convertis en produits d'un point d'ébullition de moins de 370°C.

3. Procédé selon la revendication 2, dans lequel moins de 5% en poids des composés de la charge ayant un point d'ébullition de plus de 370°C sont convertis en produits d'un point d'ébullition de moins de 370°C.

4. Procédé selon l'une quelconque des revendications 1 à 3, dans lequel les conditions d'hydroisomérisation comprennent une température comprise entre 250 et 350°C, une pression partielle d'hydrogène comprise entre 30 et 60 bar et une vitesse spatiale horaire pondérale comprise entre 0,5 et 5 kg/l/h.

5. Procédé selon l'une quelconque des revendications 1 à 4, dans lequel le métal noble est du platine, du palladium ou une combinaison desdits métaux.

6. Procédé selon l'une quelconque des revendications 1 à 5, dans lequel le support de silice - alumine amorphe possède une macroporosité de l'ordre de 5% en volume à 50% en volume, où la macroporosité est définie comme étant le pourcentage en volume des pores ayant un diamètre de plus de 100 nm.

7. Procédé selon la revendication 6, dans lequel la macroporosité est comprise entre 10 et 40% en volume.

8. Procédé selon l'une quelconque des revendications 1 à 7, dans lequel le support de silice - alumine amorphe comprend de l'alumine en une quantité de l'ordre de 2 à 75% en poids.

9. Procédé selon la revendication 8, dans lequel la teneur en alumine est de 10 à 60% en poids.

10. Procédé selon l'une quelconque des revendications 1 à 9, dans lequel le volume total de pores du support est de l'ordre de 0,6 à 1,2 ml/g.

11. Procédé selon l'une quelconque des revendications 1 à 10, dans lequel la charge d'alimentation est obtenue par une synthèse de Fischer-Tropsch.

12. Utilisation d'une cire obtenue par un procédé selon l'une quelconque des revendications 1 à 11 en tant que composant solidifiant dans un adhésif thermofusible.

13. Utilisation d'une cire obtenue par un procédé selon l'une quelconque des revendications 1 à 11 en tant que lubrifiant dans le traitement de PVC.

14. Utilisation d'une cire obtenue par un procédé selon l'une quelconque des revendications 1 à 11 en tant qu'adjuvant de brillance dans une composition cosmétique.
